

# United States Patent

[19]

Gilbert et al.

[11] 3,730,192

[45] May 1, 1973

[54] **METHOD FOR INHIBITING STAINING  
OF ELECTRODEPOSITED COATINGS  
FORMED IN A CYANIDE CONTAINING  
BATH**

[76] Inventors: **Lloyd O. Gilbert**, 824 E. Central Pk., Davenport, Iowa 52803; **John S. Finney**, 1441 Bennett, Warson Woods, Mo. 63122

[22] Filed: **Jan. 25, 1971**

[21] Appl. No.: **109,658**

[52] U.S. Cl. .... **134/2, 21/2.5 R, 134/27,**  
134/29, 134/42, 204/35 R, 210/59

[51] Int. Cl. .... **C23b 1/24, C23g 1/26**

[58] Field of Search..... **134/2, 42, 26, 27,**  
134/29; 21/2.5; 210/59; 204/35 R

[56] **References Cited**

## UNITED STATES PATENTS

|           |         |                  |            |
|-----------|---------|------------------|------------|
| 2,648,626 | 8/1953  | Buser            | 204/35 R X |
| 2,958,610 | 11/1960 | Ramirez et al.   | 134/29 X   |
| 3,105,822 | 10/1963 | Karabinos et al. | 134/42 X   |

|           |         |               |         |
|-----------|---------|---------------|---------|
| 3,475,219 | 10/1969 | Lancy         | 134/27  |
| 3,505,217 | 4/1970  | Morico        | 210/50  |
| 3,592,774 | 7/1971  | Altenschopfer | 134/2 X |

## FOREIGN PATENTS OR APPLICATIONS

|           |         |               |        |
|-----------|---------|---------------|--------|
| 1,184,594 | 12/1964 | Germany       | 210/59 |
| 909,596   | 10/1962 | Great Britain | 21/2.5 |

## OTHER PUBLICATIONS

F. Pearlstein et al., "Heat Resistant Chromate Conversion Coatings," *Plating*, April 1968, pp. 345-346.

Primary Examiner—Barry S. Richman

Attorney—Harry M. Saragovitz, Edward J. Kelly and Herbert Berl

[57] **ABSTRACT**

A method for inhibiting the staining of electrodeposited coatings which have been formed in a cyanide containing bath comprising the contacting of the coated objects with an aqueous solution of an aldose sugar.

**7 Claims, No Drawings**

**METHOD FOR INHIBITING STAINING OF  
ELECTRODEPOSITED COATINGS FORMED IN A  
CYANIDE CONTAINING BATH**

The invention described herein may be manufactured, used, and licensed by or for the Government for governmental purposes without the payment to us of any royalty thereon.

The invention relates to a method of inhibiting the staining of electrodeposited coatings which have been formed in a cyanide containing bath.

It is often desired to coat porous objects such as castings, sintered metals and assemblies having unsealed faying surfaces with copper, zinc, cadmium, gold, silver or other metals plated from a cyanide solution. During the cleaning process prior to and during the electrodeposition, solution enters the crevices, and fills voids in the porous structures. Subsequent to plating and rinsing, remaining hygroscopic solution residues pick up water forming a cyanide solution which bleeds onto the plated surface where it causes corrosion and generally unsightly staining of the metal deposit. This phenomena is known in the trade as "spotting out."

While the destruction of the cyanide film may be accomplished using other agents such as an aqueous solution rinse of a halogen, e.g., chlorine, bromine or iodine, these materials in themselves produce undesirable corrosion of the metal surfaces, if retained thereon. In addition, the discharge into the stream of the rinse containing metal halides and metal cyanide residues contribute to water pollution.

We have discovered that the undesired residues of a cyanide containing electroplating bath may be removed by rinsing the objects with an aqueous solution of an aldose sugar, e.g., talose, galactose, idose, glucose, mannose, glucose, altrose and allose. When the cyanide laden parts are introduced into a water solution of, e.g., glucose, the cyanide reacts with the sugar to form sodium heptagluconate, an excellent sequestrant, which chelates the nearby metal ions. This action reduces the corrosivity of the residues and also the toxicity of the waste water. It should be noted that this glucose treatment may be applied prior to plating as well as subsequent thereto. This is particularly applicable where the preplating treatment includes in the conditioning solution, a dilute concentration of sodium cyanide.

It is an object of this invention to provide and disclose a method for inhibiting the staining of electrodeposited coatings which have been formed in a cyanide containing bath.

It is a further object of this invention to provide and disclose an improved method for inhibiting the corrosion of electrodeposited coatings without contributing to the pollution of streams upon the discharge of the effluent rinse material.

Other objects and a fuller understanding of the invention may be ascertained by referring to the following description and claims.

The present invention is illustrated with a description of the method utilized to plate bronze bearings with cadmium to produce a plated surface free from staining. The sintered bronze bearings are first subjected to the vapors of a boiling halocarbon, e.g., trichloroethylene, in a suitable degreaser to remove oils and soil. Treatment in the vapors may be followed with

immersion in a vessel of boiling halocarbon solvent with or without applied ultrasonic agitation, followed by a short period of exposure to the halocarbon vapors to produce final rinsing action. Oxides or other

5 tarnishes are then removed by subjecting the sintered bronze to alternate anodic and cathodic polarization in an aqueous solution consisting of 3 pounds of a salt mixture of two parts caustic soda, one part tetrasodium ethylenediamine tetracetate and one part sodium cyanide per gallon of water, maintained at a temperature of up to 120° F. A current density of 50 amperes per square foot is utilized with alternate reversal of the polarity of the work pieces, i.e., 5 seconds positive - 10 seconds negative. The bearings are then removed while the polarity is positive, rinsed thoroughly in stagnated water followed by a rinse in a stagnated rinse solution containing 1-5 ounces of an aldose sugar, e.g., glucose, per gallon of water.

10 The bearings are then transferred to a cadmium plating bath which contains 4.0 ounces of cadmium oxide and 13.1 ounces of sodium cyanide per gallon of solution. The plating bath is maintained at a temperature of around 85° F. A current density (cathode) of 30 amperes per square foot is utilized. A deposit of 0.001 inch thickness is obtained in a period of approximately 20 minutes.

15 When the desired thickness of deposit has been obtained, the plated parts are rinsed in an aqueous solution of glucose. Concentration of the sugar in the solution may be in an amount of 1 to 110 ounces per gallon of water and must be maintained so as to provide an excess of sugar beyond that amount stoichiometrically equivalent to the quantities of sodium cyanide being carried into the rinse on the surface and in the pores of the parts being plated. The temperature of this aldose sugar solution may range from below ambient temperature to the boiling point thereof, e.g., 50°-212° F. A temperature of 150° F was utilized in the present illustration. Elevated temperatures accelerate the corrosion or staining inhibiting reactions and therefore are favored.

20 The glucose treated plated objects are then rinsed in cold running water and dried. When extremely porous objects are being plated, repeated alternate immersion in the hot aldose sugar solution and in cold water, with a final rinse in cold water, has been found to be more effective than a single treatment in the sugar solution followed by a cold water rinse.

25 Among the many advantages of the present invention are that; no toxic residues are left on the surface of the plated part; no toxic rinse water disposal problems are encountered, and both the aldose sugar and its reaction products with sodium cyanide, i.e., sodium heptagluconate, are totally biodegradable. In addition, both the sugar and the heptagluconate are sequestrants and therefore any residue which may remain on the surface tends to suppress the formation of ionized metallic salts thus eliminating the tendency toward stains and localized "spotting out."

30 Although we have described our invention with a certain degree of particularity, we wish it to be understood that we do not desire to be limited to the exact treatment shown and described, for obvious modifications will occur to a person skilled in the art.

Having described our invention, we claim:

1. A method for inhibiting the staining of electrodeposited coatings selected from the group consisting of copper, zinc, cadmium, gold, silver, and tin, on structures which have been electroplated in a cyanide containing bath comprising the contacting of the coated objects with an aqueous solution of an aldose sugar and thereafter rinsing said objects with water, the concentration of aldose sugar being sufficient to provide an excess of sugar beyond that stoichiometrically equivalent to the quantities of cyanide being carried into the rinse on the surface and in the pores of the objects being coated.

2. A method in accordance with claim 1 wherein the coating is cadmium.

3. A method in accordance with claim 1 wherein the electrodeposited coatings are subjected to repeated al-

ternate immersion in a hot aldose sugar solution and rinse water.

4. A method in accordance with claim 1 wherein the aldose sugar is selected from the group consisting of talose, galactose, idose, gulose, mannose, glucose, allose and allose.

5. A method in accordance with claim 4 wherein the sugar is glucose.

6. A method in accordance with claim 1 wherein the aqueous sugar solution is maintained at a temperature of about 50° to 212° F.

7. A method in accordance with claim 6 wherein the aqueous sugar solution is maintained at a temperature of around 150° F.

\* \* \* \* \*

20

25

30

35

40

45

50

55

60

65